

## UNITED STATES PATENT OFFICE

1,926,630

## ASPHALT COATED SHELL

William R. Parker and Willie L. Holbrook,  
Houston, Tex.No Drawing. Application June 14, 1932  
Serial No. 617,253

## 1 Claim. (Cl. 106—31)

This invention relates to a process or method for making an asphalt coated shell adapted for use in road building, road surfacing, sidewalks, driveways, garage floors, warehouse floors, and 5 for any other suitable purpose.

An object of this invention is to provide a process for producing asphalt coated shell consisting of washing, screening, heating and spraying so that it may be completely prepared and 10 mixed at the factory and stored and handled in bulk prior to use.

A further object of this invention is to provide a method for producing an asphalt coated shell consisting of washing the mud shell obtained 15 from a dead shell reef or the like, eliminating all foreign substances and reducing the shell particles to a uniform size.

Hitherto, shell and asphalt surfacing has been made by laying the shell on a base and applying 20 the asphalt to it, and without washing the shell to remove the foreign and deteriorating substances; in such processes it is necessary to obtain the mixing and combination at and during the construction, in order to avoid solidification.

This invention provides a method for making a material which may be entirely prepared and 25 mixed at the factory and stored in bulk ready for use. This material being made by a special process of washing, screening, heating and spraying.

Other objects will appear from the following detailed description of the invention.

The fundamental material used in this process is a mud shell, ordinarily dredged from a dead 35 shell reef by a hydraulic dredge or other means, after which it is put through a washing process.

The first step in the process consists of passing through a dewatering box which gravitates out 40 75% of the muddy water; then the material is run over a mechanically operated vibrating screen where clean water at about 10 pounds pressure is sprayed on it.

The vibrating screen serves to keep the shell in 45 constant motion by severely vibrating it, maintaining it loose and agitated so that the clean water comes in contact with every particle of shell, and at the same time grades it by causing all the material that is deteriorated and too fine for use to pass off with the washing water which 50 flows through the finest screen on the lower deck of the vibrator.

The constant vibrating and agitating of the shells against each other is necessary to leave a 55 rough surface on the shell particles to make them adhesive for the asphalt treatment.

After the shell has passed over the vibrating screen, it is discharged into a special device known as a water conveyor which has clean running water in it and serves to give the shell the final washing and also to convey it to the storage bin or pile. The shell is agitated several times 60 after it is taken out of the storage pile and before it goes into the heat treatment. This agitation allows the air to come into contact with all of the shell; the action of the air oxidizes the shell 65 causing a thin coating to form thereon.

The shell then passes through a specially designed heating and mixing apparatus having a centrifugal motion and at the same time is severely agitated. After the shell has reached a 70 suitable temperature of about 200 degrees F. and a rough adhesive surface provided, the refined asphalt or bituminous material of about the same temperature is sprayed on the shell in sufficient quantity and with sufficient pressure to 75 coat the shell thoroughly, using from approximately 10 to 25 gallons of refined asphalt or bituminous material per ton of shell, depending on the purpose for which it is to be used or the richness desired.

After the shell has passed through the heating and mixing process it may be applied to the road surface or wherever it is to be used while hot, or, if it is so desired, the shell may be placed in a storage pile, or loaded in cars of a suitable type 80 for transportation to the place where it is to be used. The process of oxidation and heating functions to make the refined asphalt or bituminous material hard and the sudden change in 85 temperature serves to dry it. This leaves the 90 shells with a dry coat of refined asphalt or bituminous material and the shell will not bind together or set until it has been spread in layers of the desired thickness on the surface for which it has been prepared and sufficiently compressed 95 by tamping or rolling until thoroughly compact. It may be used for traffic or for whatever purpose it has been prepared immediately after it has been tamped or rolled.

The material produced by this method makes 100 a surface that is dust and water proof. It will not crack or crawl for the reason that the refined asphalt or bituminous material binds it together after it has been compressed, and after it has been in use for a few days, oxidation and traffic causes a hard smooth surface to form on top, making a seal adapted to keep out all moisture, and the refined asphalt or bituminous material in a live state thereby maintaining the shell in a perfect state of preservation. If it is so 105 110

desired, a thin layer of pea gravel or sharp sand may be poured or spread over the top surface and rolled or tamped into the shell asphalt.

What we claim is,

5 A method for making a road surface covering adapted to be completely prepared and mixed at the factory, stored and handled in bulk ready for use, consisting of washing and separating mud shell material, agitating the shell portions

against each other for forming a rough adhesive surface thereon, spraying hot bituminous material on the shell until thoroughly coated and while both are heated to about 200° F., and then suddenly exposing the shell to cool air for drying and hardening the bituminous material, thereby producing coated shell.

WILLIAM R. PARKER.

WILLIE L. HOLBROOK.

80

85

10

15

90

20

95

25

100

30

105

35

110

40

115

45

120

50

125

55

130

60

135

65

140

70

145

75

150